

# UNITED STATES PATENT OFFICE.

JAMES FARRELL, OF CLEVELAND, OHIO.

## PROCESS OF MAKING CARBONIZING COMPOUNDS.

1,374,642.

Specification of Letters Patent. Patented Apr. 12, 1921.

No Drawing.

Application filed May 5, 1920. Serial No. 378,988.

To all whom it may concern:

Be it known that I, JAMES FARRELL, a citizen of the United States, resident of Cleveland, county of Cuyahoga, and State 5 of Ohio, have invented new and useful Improvements in Processes of Making Carbonizing Compounds, of which the following is a specification, the principle of the invention being herein explained and the best 10 mode in which I have contemplated applying that principle, so as to distinguish it from other inventions.

My invention relates to metal treatment, and particularly to processes of making 15 compounds by which all metals, preferably iron and steel, may be carbonized. The invention relates particularly to the making of compounds utilized for case-hardening iron and steel.

20 The following description sets forth in detail certain steps embodying my invention, the disclosed steps, however, constituting but one of the various forms in which the principle of the invention may be applied.

25 In carrying out my improved process, I utilize any inactive carbonaceous substance. By this I mean all forms of carbon which can be charred or burned. This includes all 30 forms of carbon except graphite and diamond. These forms, which I use, I term, generally, "amorphous carbon," and they are illustrated by such materials as charcoal, coke, wood shavings, saw-dust, wood 35 bark, peat, bone, etc. I first remove from said inactive carbonaceous material substantially all of the moisture contained therein.

30 This drying operation is effected in a closed boiler heated by steam coils to substantially three hundred and three (303) degrees Fahrenheit, the steam pressure being substantially fifty-five (55) pounds, combined with the step of effecting a vacuum in the boiler of about twenty-eight and one-half (28½) inches mercury. As stated above, this process removes substantially all of the moisture from the inactive carbonaceous material. By actual tests, I have 45 removed by this process from amorphous carbon, such as charcoal, seven per cent. (7%) by weight moisture and from coke six per cent. (6%) by weight. By a further step of my process, I impregnate the inactive carbonaceous material dried as stated above, with an energizing substance such as

lime, soda ash, sodium carbonate, barium carbonate, calcium carbonate, or any other suitable material or combination of materials, which, when added to the inactive carbonaceous material, renders the latter active for carbonizing purposes. This impregnating is effected under a steam pressure from fifty to one-hundred and fifty pounds in any suitable inclosed boiler, the 60 contents of the latter being heated to from one hundred to three hundred degrees Fahrenheit, the temperature and pressure depending within certain limits upon the density of the boiler contents. Preferably, I 65 utilize for this impregnating step a pressure of about eighty pounds and a temperature of about two hundred and eighty degrees Fahrenheit. This impregnation may take place by either a dry or a wet process, in 70 the case of the wet process lime being generally used in combination with some other energizing agent. However, if the impregnation is effected by a wet process, it is then necessary to dry the carbonizing compound 75 again; otherwise, it would steam the pots in the furnace during the packing and carbonizing period. By actual tests, I have impregnated charcoal from which seven per cent. by weight moisture has been removed 80 by the vacuum process, with one hundred and thirty-nine per cent. by weight of the energizing agent, of which thirty per cent. remained after the second drying. This second drying process is also a vacuum 85 process. Furthermore, I have impregnated coke, from which six per cent. by weight of moisture has been removed, by the vacuum process, with sixty per cent. by weight of the energizing substance, of which nineteen to twenty per cent. remained after the 90 second drying.

95 My improved process results in the formation economically of a compound which is extremely effective in the efficient case-hardening of iron and steel.

What I claim is:

1. The process of making carbonizing compounds consisting in, removing substantially all the moisture from carbonaceous 105 material by vacuum process and then impregnating the material with an energizing agent under fifty (50) to one hundred and fifty (150) pounds pressure and a temperature of from 100° to 300° Fahrenheit. 110

2. The process of making carbonizing compounds consisting in, removing substan-

tially all the moisture from carbonaceous material by subjecting the same to a vacuum of approximately twenty-eight and one-half (28 $\frac{1}{2}$ ) inches mercury and then impregnating 5 the material with sodium carbonate under fifty (50) to one hundred and fifty (150) pounds pressure and a temperature of from 100° to 300° Fahrenheit.

3. The process of making carbonizing 10 compounds consisting in, removing substantially all the moisture from amorphous carbon by subjecting the same to a vacuum process while heated to substantially three hundred and three (303) degrees Fahrenheit, and under substantially fifty-five (55) 15 pounds steam pressure and then impregnating the dried carbon with sodium carbonate and lime by confining the same with the impregnating materials in an inclosed boiler 20 under fifty (50) to one hundred and fifty (150) pounds pressure and a temperature of from 100° to 300° Fahrenheit.

4. The process of making carbonizing 25 compounds consisting in, removing substantially all the moisture from carbonaceous material by vacuum process and then impregnating the material with an energizing agent.

5. The process of making carbonizing 30 compounds consisting in, removing substantially all the moisture from charcoal by vacuum process; impregnating the charcoal thus dried with substantially one hundred forty (140) per cent. by weight of a solution 35 of lime and sodium carbonate; and then drying the impregnated charcoal, whereby the same remains impregnated with

substantially thirty (30) per cent. by weight of energizing agent.

6. The process of making carbonizing 40 compounds consisting in, removing substantially six (6) per cent. by weight of moisture from coke by vacuum process; impregnating the coke thus dried with substantially sixty (60) per cent. by weight of a solution 45 of lime and sodium carbonate; and then drying the impregnated coke, whereby the same remains impregnated with substantially twenty (20) per cent. by weight of energizing agent. 50

7. The process of making carbonizing compounds consisting in, removing substantially all the moisture from carbonaceous material by vacuum process and then impregnating the material with an energizing 55 agent under pressure.

8. The process of making carbonizing compounds consisting in, removing substantially all the moisture from amorphous carbon by subjecting the same to a vacuum 60 process while heated to a temperature of substantially three hundred and three (303) degrees Fahrenheit and under substantially fifty-five (55) pounds steam pressure and then impregnating the dried carbon with an 65 energizing agent by confining the same with the impregnating materials in an inclosed boiler under substantially eighty (80) pounds pressure and a temperature of substantially two hundred eighty (280) degrees Fahrenheit. 70

Signed by me, this 3d day of May, 1920.

JAMES FARRELL.